

## UNITED STATES PATENT OFFICE

1,954,750

## MANUFACTURE OF PATENT LEATHER

Horace H. Hopkins, Ridley Park, Pa., assignor to  
 E. I. du Pont de Nemours & Company, Wil-  
 mington, Del., a corporation of Delaware

No Drawing. Application December 18, 1930,  
 Serial No. 503,227

## 7 Claims. (CL. 91—70)

This invention relates to the manufacture of patent leather and more particularly to an improved outer or top coating for patent leather finishes.

One of the chief disadvantages in the manufacture of patent leather resides in the long sunning treatment required to dry and remove the tack after completion of the process. While different manufacturers carry out the process according to their own unique procedure, which may involve trade secrets, the following two methods may be considered essentially typical of the methods commonly used; all of which methods necessitate the expensive sunning treatment referred to.

One widely used method of manufacturing patent leather is substantially as follows:

A heavy consistency first coat of a mixture of japanner's oil (bodied linseed oil) and a pigment is applied to the leather and rubbed in with the hands. Two or three coats of clear varnish, consisting of japanner's oil thinned with naphtha, are next applied. These coats of clear varnish, as well as the first mentioned coating of pigment-ed japanner's oil, are applied with a sponge and are dried overnight at about 90°—100° F. A final coat of japanner's varnish (strongly boiled linseed oil) is now flowed on, and the leather baked in a japanner's oven for about sixteen hours at approximately 160° F. To remove the final tack from the top coat varnish it must be exposed to sunlight for at least five hours, the only possible alternative for sunning being the very expensive ultraviolet irradiating equipment which is rarely used in this country. In spite of the sunning the finish is often still tacky or sticky at slightly elevated temperatures and is often waxed or packed in waxed paper to prevent sticking during shipping.

A second method, sometimes used in the manufacture of patent leather, is to apply a finish in which pyroxylin is utilized. The pyroxylin finish, does not require quite as much sunning, and dries slightly better, but it is considerably more expensive than the oil type finish. In this case the entire finish consists of a mixture of pyroxylin and japanner's oil, thinned to a suitable consistency for applying with a blunt edged metal knife. Four or five coats of this mixture are applied, each being dried overnight at about 90° F.

Even in this process, however, the final coat contains no pyroxylin, and consists entirely of japanner's varnish as in the first method, and must be sunned to remove tackiness.

The two methods described produce similar types of patent leather, both of which have two extremely important drawbacks. The first is the fact that sunning must be resorted to. It can be readily seen that any manufacturing process that depends on the weather as completely as does this one, is subject to many uncertainties. There are times, especially during the winter months, when production may be held up for weeks due to the absence of sun which is necessary for the final operation. In the winter, when the weather is liable to be most cloudy, the leather needs a longer time of sunning due to the smaller amount of ultraviolet light in the sun's rays at that season. In addition to the difficulties involved in the manufacturing process, a second disadvantage resides in the defects inherent in the product itself. In this connection may be mentioned the fact that these finishes are subject to rapid embrittling which produces large unsightly cracks in the patent leather product.

This invention has as an object a method of manufacturing patent leather which does not require sunning or exposure to ultraviolet light. Another object is the production of patent leather having a top coat finish which gives a more permanent retention of flexibility, and hence elimination of the early cracking of the finish, so common in previously known types of patent leather.

These objects are accomplished by the following invention in which a varnish comprising a solution of a synthetic resin of the polyhydric alcohol-polybasic acid type, modified with a drying oil, with or without small proportions of other ingredients, is applied as a top coat in the manufacture of patent leather.

In accordance with the practice of the present invention the final coat of oil varnish applied in the processes referred to above, is omitted and in lieu thereof is applied a top coat of a solution of a drying oil modified polyhydric alcohol-polybasic acid resin. This coating may be a solution in any suitable solvent for the particular resin or resins used, and may contain small quantities of additional ingredients, which in some way enhance the value of the coating.

53

60

65

70

75

80

85

90

95

100

Polyhydric alcohol-polybasic acid resins modified in any desired proportions with drying oils may be used, but resins of the following compositions, expressed in terms of the reacting constituents, have been found to be especially suitable:

## Resin A

|                    | Parts by weight |
|--------------------|-----------------|
| 10 Glycerol        | 12.6            |
| Phthalic anhydride | 29.7            |
| Linseed oil        | 57.7            |

## 15 Resin B 100.0

|                       | Parts by weight |
|-----------------------|-----------------|
| Glycerol              | 12.60           |
| 20 Phthalic anhydride | 29.70           |
| Linseed oil           | 28.85           |
| Chinawood oil         | 28.85           |
|                       | 100.00          |

25 The glyceryl phthalate in the preceding two resins constitutes about 40% by weight of the resin.

## Resin C

|                    | Parts by weight |
|--------------------|-----------------|
| 30 Glycerol        | 10.8            |
| Phthalic anhydride | 26.2            |
| Perilla oil        | 63.0            |
|                    | 100.0           |

This resin contains about 35% by weight of glyceryl phthalate.

## Resin D

|                    | Parts by weight |
|--------------------|-----------------|
| 40 Glycerol        | 14.1            |
| Phthalic anhydride | 33.3            |
| Soya bean oil      | 52.6            |
|                    | 100.0           |

This resin contains about 45% by weight of glyceryl phthalate.

50 The foregoing resins may be made by any of the methods commonly used for the manufacture of oil modified polyhydric alcohol-polybasic acid resins. As indicated in the examples the preferred polyhydric alcohol is glycerol and the preferred polybasic acid is phthalic anhydride. Other polyhydric alcohols and polybasic acids, known by those skilled in the art of manufacturing this type of resin, may be used. Among the polyhydric alcohols commonly used are pentaerythritol, polyethylene glycol, etc. Examples of other suitable polybasic acids are, succinic acid, fumaric acid, maleic acid, and adipic acid.

Instead of drying oils, the equivalent amount of drying oil acids may be used in manufacturing these resins as understood by those skilled in the art. The drying oil mentioned in the claims refers, therefore, to the drying oil acids as well as to the drying oil itself. Additional ingredients which may be incorporated with the resins in small amounts (for example, up to 10%) are rosin or other resin acids, mixtures of monohydric (e. g. benzyl) or polyhydric alcohols (e. g. ethylene glycol) as well as substituted polyhydric alcohols such as glycol ethers. Certain high boiling organic substances such as xylol, solvent naphtha,

terpenes, turpentine substitutes, and many others may be incorporated. If desired certain metallic driers, such as cobalt, lead, manganese, or iron linoleate may be used to speed up the drying of the finish.

80 The coating may be applied to the flexible base material by brushing, spraying, swabbing, or by any suitable method, preferably at such a consistency that the solution as applied contains about 40-60% of solid material. The leather is then baked in order to suitably dry the film, about 10 to 20 hours at about 150 to 175° F. having been found suitable.

85 This invention has several important advantages over the production of patent leather by the methods heretofore used. One of these advantages relates to the manufacture of the patent leather and resides in the fact that no sunning is necessary because the hardening, in the present case, is accomplished by baking. This is possible with my new finish because, while the previously used oil films "set up" almost entirely by oxidation, the resin films of the present invention harden by a combination of oxidation and polymerization, the latter process being appreciably hastened by heat.

90 Because of the exceptional toughness and lasting flexibility of the film yielded by the particular type of resin used, the new finish retains its flexibility for a considerably longer period than the old type of finish, and thus remains free from cracks for a longer period of time.

95 A further advantage resides in the fact that my new patent leather is almost entirely free from the residual tackiness which is often present in patent leather even after sufficient sunning. This feature is especially important if the leather is to be packed for shipment through any great distance, and especially if it is to be subjected to elevated temperatures, as in shipping 105 through warm regions. An entire shipment of excellent quality patent leather is sometimes lost because the packed sheets have stuck together, and cannot be separated without tearing great holes in the coating.

100 As many apparently widely different embodiments of this invention may be made without departing from the spirit and scope thereof, it is to be understood that I do not limit myself to the specific embodiments thereof except as defined in the appended claims.

105 I claim:

110 1. A process of manufacturing patent leather which comprises subjecting leather to treatment with a composition comprised of japanner's oil, applying over the coating or coatings applied in such treatment a coating comprising a drying oil modified polyhydric alcohol-polybasic acid resin, and baking to harden the resin coating.

115 2. A process of manufacturing patent leather which comprises subjecting leather to treatment with a composition comprising japanner's oil, applying over the coating or coatings applied in such treatment a coating comprised of the resinous reaction product of glycerol, phthalic anhydride, and a drying oil.

120 130 3. A step in a process for manufacturing patent leather which comprises applying a coating of a drying oil modified glyceryl phthalate resin containing in combined form from about 52% to 63% drying oil over the previously applied undercoats, and baking the product.

135 145 4. In the manufacture of patent leather products the steps of applying a pyroxylin-oil under-

coat and applying a top coat of oil modified polyhydric alcohol-polybasic acid resin.

5. In the manufacture of patent leather products the steps of applying a pyroxylin-containing undercoat and applying a top coat of oil modified polyhydric alcohol-polybasic acid resin.

6. A patent leather product having an undercoat comprising a dried film of pyroxylin-oil

composition and a top coat of oil modified polyhydric alcohol-polybasic acid resin.

7. A patent leather product having a flexible base having an undercoat comprising pyroxylin and a top coat of oil modified polyhydric alcohol- 80 polybasic acid resin.

HORACE H. HOPKINS.

|    |     |
|----|-----|
| 10 | 85  |
| 15 | 90  |
| 20 | 95  |
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 |     |
| 75 |     |